

## UNITED STATES PATENT OFFICE

FREDERICK M. BECKET, OF NEW YORK, N. Y., ASSIGNOR TO ELECTRO METALLURGICAL COMPANY, A CORPORATION OF WEST VIRGINIA

## STAIN-RESISTING ALLOY

No Drawing.

Application filed April 16, 1930. Serial No. 444,876.

This invention relates to stain-resisting alloys containing, as essential constituents, the metals iron, chromium, manganese and copper.

5 In an application bearing Serial No. 435,-957, filed by me on March 14, 1930, I have described alloys consisting essentially of iron, chromium and manganese; and I have shown that within the limits of composition 10 given in the said application, the alloys combine deep-drawing properties with high resistance to staining and corrosion, and exhibit this combination of properties not only when quenched from temperatures of about 15 1000° C. to 1150° C., but also when air-cooled from like temperatures. The alloys discussed in my said prior application contain about 16%-22% of chromium; about 20 5%-15% of manganese; and up to about 0.3% of carbon. When the carbon is below about 0.12% the alloys are especially soft and ductile, but not quite so strong as when the carbon is higher.

I have now found that copper may be 25 added to the alloys of my prior application giving new alloys with desirable properties. Such new alloys, when the copper content is suitably adjusted, are strain-resistant in approximately the same degree as the alloys 30 of my prior application; and while the copper tends slightly to increase the hardness of the alloys, an appropriate addition of copper raises the Erichsen value and gives such a combination of physical properties as to 35 indicate excellent deep-drawing qualities,—an inference which is confirmed by actual drawing tests.

By adding copper to the alloys of my prior application it is possible with a medium 40 manganese content, say in the vicinity of 8%, to equal or, it seems probable, distinctly to surpass the drawing qualities obtainable without copper by incorporating a higher proportion of manganese. The present invention therefore offers the possibilities of 45 providing still better alloys than those described in my prior application, and of lowering the cost of the alloys by replacing a 50 part of the manganese with the cheaper metal copper.

Although I have done a large amount of experimental work on the new alloys it has not been feasible to test all possible compositions, and it is deemed unsafe in this field to permit the conclusions to wander far from 55 the experimental basis. I therefore refrain from setting precise limits on the additions of copper which may be useful. Such limits are not of the essence of the invention, and in practice limiting values of the copper content would be avoided in view of the impossibility in even the best metallurgical practice of working to precise limits. With this qualification it may be said that the useful copper range lies between the approximate 60 limits of 0.25% and 2.5%. When the copper content is too high, the alloy tends to become hot-short. With the manganese at 8% or less the copper may rise to 2.5% and perhaps beyond, but with higher manganese percentages, in the vicinity of 14%, 2.5% of copper 65 seems to be excessive, or at least not to be recommended. Alloys containing 3% of copper with as little as 6% of manganese 70 were definitely hot-short, and broke up during forging.

As stated above, the chromium may be varied through about the range (16%-22%) given in my prior application, but my experimental work has been largely confined to 80 compositions containing about 18% of chromium, it having been established in prior work with iron-chromium, iron-chromium-nickel, and iron-chromium-manganese alloys 85 that a chromium percentage not far from this value is in most cases quite satisfactory, and found in the present investigation that about 18% of chromium is equally satisfactory 90 in the copper-containing alloys.

The carbon percentages set out in my prior application, viz. not more than about 0.3%, and preferably not more than 0.12 are also recommended for the iron-chromium-manganese copper alloys of deep-drawing quality.

The following tabulation shows the composition of specific alloys within my invention, and gives the numbers obtained in 100

physical tests carried out on the respective alloys as quenched from 1050°-1150° C.:

| 5  | C    | Cr    | Mn   | Cu   | Yield point | Max. stress | Elongation in 2in. | Reduction of area | Erichsen | Brinell |
|----|------|-------|------|------|-------------|-------------|--------------------|-------------------|----------|---------|
|    |      |       |      |      |             |             | Per cent           |                   |          |         |
| 10 | 0.10 | 17.20 | 9.78 | 0.52 | 47,000      | 116,000     | 40.0               | 38.8              | 11.4     | 179     |
|    | 0.08 | 19.25 | 8.68 | 1.10 | 47,000      | 127,000     | 40.5               | 41.0              | 10.8     | 179     |
|    | 0.12 | 17.07 | 8.69 | 1.12 | 52,300      | 106,600     | 47.0               | 53.0              | 11.4     | 179     |
|    | 0.10 | 16.33 | 8.31 | 1.64 | 43,000      | 111,000     | 40.0               | 42.5              | 11.1     | 163     |
|    | 0.09 | 16.38 | 8.64 | 2.12 | 48,900      | 89,900      | 45.5               | 59.7              | 10.6     | 163     |
|    | 0.10 | 17.50 | 8.50 | 2.50 | 54,000      | 92,000      | 48.0               | 70.7              | 10.4     | 159     |

15 As in the case of the alloys of application Serial No. 435,957 the chromium percentages which appear most promising fall between the approximate limits of 17% and 21%. Since the addition of copper permits the 20 manganese percentage to be lowered, the preferred range for manganese in the copper-containing alloys is defined by the approximate limits 6% and 10%.

I claim:—

- 25 1. A stain-resisting iron-base alloy containing chromium about 16% to 22%; manganese about 5% to 15%; and carbon, the carbon content being not more than 0.3%; copper about 0.25% to 3.0%; with the balance substantially iron.
- 30 2. A stain-resisting iron-base alloy having deep-drawing properties and containing chromium about 16% to 22%; manganese about 5% to 15%; copper about 0.25% to 2.5%; and carbon, the carbon content being not more than 0.3%; with the balance substantially iron.
- 35 3. A stain-resisting iron-base alloy having deep-drawing properties and containing chromium about 16% to 22%; manganese about 5% to 15%; copper about 0.25% to 2.5%; and carbon, the carbon content being not more than 0.12%; with the balance substantially iron.
- 40 4. A stain-resisting iron-base alloy having deep-drawing properties and containing chromium about 16% to 22%; manganese about 6% to 10%; copper about 0.25% to 2.5%; and carbon, the carbon content being not more than 0.12%; with the balance substantially iron.
- 45 5. A stain-resisting iron-base alloy having deep-drawing properties and containing chromium about 17% to 21%; manganese about 6% to 10%; copper about 0.25% to 2.5%; and carbon, the carbon content being not more than 0.12%; with the balance substantially iron.

In testimony whereof, I affix my signature.

FREDERICK M. BECKET.